



US005912607A

# United States Patent [19]

Kalsi et al.

[11] Patent Number: 5,912,607

[45] Date of Patent: Jun. 15, 1999

[54] FAULT CURRENT LIMITING  
SUPERCONDUCTING COIL[75] Inventors: **Swarn S. Kalsi; Gregory L. Snitchler**,  
both of Shrewsbury, Mass.; **Jeffrey M. Seuntjens**, Singapore, Singapore[73] Assignee: **American Superconductor Corporation**, Westborough, Mass.

[21] Appl. No.: 08/928,901

[22] Filed: Sep. 12, 1997

[51] Int. Cl.<sup>6</sup> ..... H01F 1/00

[52] U.S. Cl. ..... 335/216; 505/705

[58] Field of Search ..... 335/216, 296-301;  
324/318-322; 505/705

## [56] References Cited

## U.S. PATENT DOCUMENTS

4,933,657 6/1990 Bessho et al. ..... 335/299  
4,939,444 7/1990 Cacheux .  
5,138,626 8/1992 Edwards et al. .5,231,074 7/1993 Cima et al. .  
5,387,891 2/1995 Nick .  
5,659,277 8/1997 Joshi et al. ..... 335/216  
5,689,223 11/1997 Demarmels et al. ..... 335/216

## FOREIGN PATENT DOCUMENTS

41 32 067 A1 5/1992 Germany .

Primary Examiner—Lincoln Donovan  
Attorney, Agent, or Firm—Fish & Richardson P.C.

## [57] ABSTRACT

A superconducting magnetic coil includes a first superconductor formed of an anisotropic superconducting material for providing a low-loss magnetic field characteristic for magnetic fields parallel to the longitudinal axis of the coil and a second superconductor having a low loss magnetic field characteristic for magnetic fields perpendicular to the longitudinal axis of the coil. The first superconductor has a normal state resistivity characteristic conducive for providing current limiting in the event that the superconducting magnetic coil is subjected to a current fault.

49 Claims, 3 Drawing Sheets





FIG. 1



FIG. 2



FIG. 3



FIG. 4



FIG. 5



FIG. 6



FIG. 7



FIG. 8



FIG. 9



FIG. 10

## FAULT CURRENT LIMITING SUPERCONDUCTING COIL

### BACKGROUND OF THE INVENTION

The invention relates to superconducting magnetic coils.

An important property of a superconductor is the disappearance of its electrical resistance when it is cooled below a critical temperature  $T_c$ . Below  $T_c$  and for a given superconductor, there exists a maximum amount of current - - - referred to as the critical current ( $I_c$ ) of the superconductor - - - which can be carried by the superconductor at a specified magnetic field and temperature. Any current in excess of  $I_c$  causes the onset of resistance in the superconductor. If the superconductor is embedded in or co-wound with a conductive matrix, any incremental current above  $I_c$  will be shared between the superconductor and matrix material based on the onset of resistance in the superconductor.

Superconducting materials are generally classified as either low or high temperature superconductors. High temperature superconductors (HTS), such as those made from ceramic or metallic oxides are typically anisotropic, meaning that they generally conduct better, relative to the crystalline structure, in one direction than another. Moreover, it has been observed that, due to this anisotropic characteristic, the critical current varies as a function of the orientation of the magnetic field with respect to the crystallographic axes of the superconducting material. Anisotropic high temperature superconductors include, but are not limited to, the family of Cu—O-based ceramic superconductors, such as members of the rare-earth-copper-oxide family (YBCO), the thallium-barium-calcium-copper-oxide family (TBCCO), the mercury-barium-calcium-copper-oxide family (HgBCCO), and the bismuth strontium calcium copper oxide family (BSCCO). These compounds may be doped with stoichiometric amounts of lead or other materials to improve properties (e.g.,  $(\text{Bi},\text{Pb})_2\text{Sr}_2\text{Ca}_2\text{Cu}_3\text{O}_{10}$ ). Anisotropic high temperature superconductors are often fabricated in the form of a superconducting tape having a relatively high aspect ratio (i.e., width greater than the thickness). The thin tape is fabricated as a multi-filament composite superconductor including individual superconducting filaments which extend substantially the length of the multi-filament composite conductor and are surrounded by a matrix-forming material (e.g., silver). The ratio of superconducting material to matrix-forming material is known as the “fill factor” and is generally less than 50%. Although the matrix forming material conducts electricity, it is not superconducting. Together, the superconducting filaments and the matrix-forming material form the multi-filament composite conductor.

High temperature superconductors may be used to fabricate superconducting magnetic coils such as solenoids, racetrack magnets, multiple magnets, etc., in which the superconductor is wound into the shape of a coil. When the temperature of the coil is sufficiently low that the HTS conductor can exist in a superconducting state, the current carrying capacity as well as the magnitude of the magnetic field generated by the coil is significantly increased.

High temperature superconductors have been utilized as current limiting devices to limit the flow of excessive current in electrical systems caused by, for example, short circuits, lightning strikes, or common power fluctuations. HTS current limiting devices may have a variety of different configurations including resistive and inductive type current limiters.

### SUMMARY OF THE INVENTION

The invention features a superconducting magnetic coil having a first superconductor formed of an anisotropic superconducting material for providing a low-loss magnetic field characteristic for magnetic fields parallel to the longitudinal axis of the coil and a second superconductor having a low loss magnetic field characteristic for magnetic fields perpendicular to the longitudinal axis of the coil (e.g., when the orientation of an applied magnetic field is perpendicular to the wider surface of a superconductor tape, as opposed to when the field is parallel to this wider surface).

In embodiments, the first superconductor has a normal state resistivity characteristic conducive for providing current limiting in the event that the superconducting magnetic coil is subjected to a current fault.

In a general aspect of the invention, the first superconductor is wound about the longitudinal axis of the coil and is formed of an anisotropic superconducting material having a first resistivity characteristic in a normal state of operation; and a second superconductor, wound about the longitudinal axis of the coil and connected to the first anisotropic superconductor, having a second resistivity characteristic, in a normal state of operation, less than the resistivity characteristic of the first anisotropic superconductor in a normal state of operation.

Among other advantages, the first superconductor has a resistivity characteristic such that, should it lose its superconducting properties (e.g., due to an increase in current) and revert back to its normally conducting state, the first superconductor resistively limits current flowing through the coil, thereby preventing damage to itself, the second superconductor, and other components connected to the superconducting magnetic coil. Thus, in one application, the superconducting magnetic coil provides reliable protection in the event of a current fault by limiting the current flowing through the coil for a time period sufficient to allow a circuit breaker to be activated or fuse to be blown, thereby preventing further current flow and potentially catastrophic damage to the superconducting magnetic coil and other components of the system. During normal superconducting operation, the coil has a low loss allowing greater current handling capability.

In another aspect of the invention, a first anisotropic superconductor is wound about the longitudinal axis of the coil and is formed as a superconducting tape, the first anisotropic superconductor configured to provide a low AC loss characteristic in the presence of magnetic fields parallel to the wide surface of the superconductor tape; and a second superconductor, different from the first anisotropic superconductor. The second superconductor is wound about the longitudinal axis of the coil and is connected to an end of the first anisotropic superconductor and configured to provide a low AC loss characteristic in the presence of magnetic fields perpendicular to the wide surface of the superconductor tape of the first anisotropic superconductor.

Embodiments of the above described aspects of the invention may include one or more of the following features.

The second superconductor is connected to an end of the first anisotropic superconductor and is configured to provide a low AC loss characteristic in the presence of perpendicular magnetic fields. The second superconductor is an anisotropic material and is in the form of a tape.

The first anisotropic superconductor is in monolithic form (i.e., in the form of a monofilament or a group of closely spaced multifilaments that are electrically fully coupled to

each other, thus acting as a monofilament). Alternatively, the monolithic-form first anisotropic superconductor tape includes a multifilament composite superconductor having individual superconducting filaments which extend the length of the multifilament composite superconductor. The multifilament composite superconductor has a resistivity characteristic, in its normal state, in a range between about 0.1 to 100  $\mu\Omega\text{-cm}$ , preferably 5 to 100  $\mu\Omega\text{-cm}$ .

The first anisotropic superconductor can also be in the form of a superconductor tape and generally has an aspect ratio in a range between about 5:1 and 1000:1. The first anisotropic superconductor may include a backing strip formed of a thermal stabilizer having a resistivity characteristic greater than about 1  $\mu\Omega\text{-cm}$ .

The second anisotropic superconductor can be a tape having multifilament composite superconductor with individual superconducting filaments which extend the length of the multifilament composite superconductor and are surrounded by a matrix forming material.

The first and second anisotropic superconductors may be wound in a layered configuration. Alternatively, the first and second anisotropic superconductors are formed of single or double pancake coils, each coil electrically connected to an adjacent coil.

In an alternative embodiment, the first and second anisotropic superconductors are wound in a "spliced arrangement". With this arrangement, a first segment of the first anisotropic superconductor extends along the longitudinal axis in a first direction toward the second anisotropic superconductor and connects to a first end of a first segment of the second anisotropic superconductor at a first junction. A second end of the first segment is connected to a second segment of the first anisotropic superconductor, the second segment extending along the longitudinal axis in second direction way from the second anisotropic superconductor.

The first and second anisotropic superconductors are high temperature superconductors.

In certain embodiments, the second superconductor constitutes a portion of the total amount of superconductor of the coil in a range between about 5% and 30%, for example, 10%.

Other advantages and features will become apparent from the following description and the claims.

#### BRIEF DESCRIPTION OF THE DRAWING

FIG. 1 is a cross-sectional side view of a superconducting coil of the invention having "pancake" coils.

FIG. 2 is a cross-sectional side view of the superconducting coil of FIG. 1 having "pancake" coils.

FIG. 3 is a side view of the superconductor tape associated with a central region of the superconducting coil of FIG. 1.

FIG. 4 is a side view of the superconductor tape of FIG. 3 having a laminated thermal backing layer.

FIG. 5 is a cross-sectional view of a multifilament composite conductor associated with end regions of the superconducting coil of FIG. 1.

FIG. 6 is an enlarged perspective view of a multistrand cable for the multifilament composite conductor of FIG. 5.

FIG. 7 is a perspective view of an alternative superconducting coil of the invention.

FIG. 8 is a cross-sectional side view of a portion of another superconducting coil of the invention.

FIG. 9 is a cross-sectional side view of a portion of a transformer having a superconducting coil of the invention.

FIG. 10 is a plot showing the RMS radial coil field as a function of the percent of the axial coil length.

#### DESCRIPTION

Referring to FIG. 1, a mechanically robust, high-performance superconducting coil assembly 5 includes an iron core 6 and a superconducting coil 8 having a central region 11 and end regions 14. As will be discussed in greater detail below, the superconductor material used to form central region 11 has characteristics different than that used to form end regions 14. In particular, central region 11 is formed with a conductor 18 (FIG. 3) having a low loss characteristic in its superconducting state, but in its normal state has a relatively high resistivity characteristic, so that central region 11 serves as a current limiting section of coil assembly 10. Thus, in the event of an electrical current fault, conductor 18 reverts to its normal, non-superconducting, state for a time sufficient to prevent coil assembly 10 from being damaged due to overheating. During the time that current is being limited by conductor 18 in its normal state, a circuit breaker or fuse can be used to open the circuit and prevent further current flow.

End regions 14 are formed of a conductor 22 (FIG. 5) which, unlike conductor 18 of central region 11, is configured to provide a low AC loss characteristic in the presence of perpendicular magnetic fields. Conductor 22 is configured in this manner because magnetic field lines emanating from superconducting magnetic coil assembly 10 at end regions 14 become perpendicular with respect to the plane of conductor 22 (the conductor plane being parallel to the wide surface of the superconductor tape) causing the critical current density at these regions to drop significantly. In fact, the critical current reaches a minimum when the magnetic field is oriented perpendicularly with respect to the conductor plane.

Referring to FIG. 2, in one embodiment, a superconducting coil 10 includes central region 11 and end region 14 formed with interconnected double "pancake" coils 12a, 12b. Central region 11 is shown here having seven separate double pancake sections 12a and each end region 14 is shown having a single pancake section 12b. Each double "pancake" coil 12a, 12b has co-wound superconductors wound in parallel which are then stacked coaxially on top of each other, with adjacent coils separated by a layer of insulation 16.

An inner support tube 17 supports the coils of central region 11 and end regions 14 with end members 20 attached to opposite ends of inner support tube 17 to compress the coils of central region 11 and end regions 14. Inner support tube 17 and end members 20 are fabricated from an electrically insulative, non-magnetic material, such as aluminum or plastic (for example, G-10).

Referring to FIG. 3, each double pancake coil 12a of conductor 18 is fabricated from an HTS anisotropic superconductor formed in the shape of a thin tape which allows the conductor to be bent around relatively small diameters and allows the winding density of the coil to be increased. A method of fabricating double pancake superconducting coils with superconducting tape of this type is described U.S. Pat. No. 5,531,015, assigned to the present assignee, and incorporated herein by reference. Conductor 18 is relatively long and has a relatively large aspect ratio in a range between about 5:1 and 1000:1. For superconductor tapes formed from the BSCCO family, the aspect range is generally between about 5:1 and 20:1 while for tapes formed from YBCO family, the aspect range is generally between

about 100:1 and 1000:1, typically about 400:1. Conductor **18** is in monolithic form, meaning that the HTS anisotropic superconductor is in the form of a monofilament **15** or a group of closely spaced multifilaments which are electrically fully coupled to each other and act as a monofilament. The monolithic form conductor **18** is not affected in the same manner as conductor **22** at end regions **14** and provides a relatively low AC loss characteristic because the magnetic fields are substantially parallel along the axis of central region **11**.

The monolithic form conductor **18** may be a rare-earth-copper-oxide family (YBCO) material such as those described in U.S. Pat. No. 5,231,074 to Cima et al., entitled "Preparation of Highly Textured Oxide Superconducting Films from MOD Precursor Solutions" which is hereby incorporated by reference. Alternatively, conductor **18** may be formed of other Cu—O-based ceramic superconductors, such as bismuth strontium calcium copper oxide family (BSCCO) which is typically in the form of a composite of individual superconducting filaments surrounded by a matrix forming material. A description of such composite superconducting tapes is described in U.S. Pat. No. 5,531,015.

Referring to FIG. 4, conductor **18** is laminated onto a thermal stabilizing backing strip **19** formed, for example, of stainless steel, nickel or other suitable alloy. Because resistive heating in conductor **18** can be high, backing strip **19** serves as a heat sink to maintain the temperature of conductor **18** within a safe level while also providing a high resistance path for current flowing through coil assembly **10**. Backing strip **19** has a resistivity characteristic greater than about 10  $\mu\Omega\text{-cm}$ . When conductor **18** is formed of YBCO material, substantially all of the current flows through backing strip **19**. On the other hand, where a composite superconductor material is used (e.g., formed of BSCCO) current can also flow through the matrix material of the composite which has a resistivity characteristic in a range between about 0.1 to 100  $\mu\Omega\text{-cm}$ .

End regions **14** are also formed of a high-temperature superconductor, but of a material different from that used to wind central region **11**. Although isotropic superconductor materials may be used, in many applications, anisotropic superconductors, such as BSCCO type composite superconductor are preferred.

Referring to FIGS. 5 and 6, end regions **14** do not have a monolithic form. Rather, conductor **22** is a thin tape **24** fabricated of a multi-filament composite superconductor having individual superconducting filaments **27** which extend substantially the length of the multi-filament composite conductor and are surrounded by a matrix-forming material **28**, typically silver or another noble metal. In other embodiments, aspected multifilament strands can be combined and are preferably twisted, for example, in the manner shown in the illustration of a multistrand cable **28** (FIG. 6). Twisting the individual multifilament strands and separating them with a matrix material having a high resistivity characteristic is important for providing the low AC loss characteristic in the presence of perpendicular magnetic fields. Details relating to the types of superconductors and their methods of fabrication suitable for use in forming conductor **22** are described in co-pending application Ser. No. 08/444,564 filed on May 19, 1995 by G. L. Snitchler, G. N. Riley, Jr., A. P. Malozemoff and C. J. Christopherson, entitled "Novel Structure and Method of Manufacture for Minimizing Filament Coupling Losses in Superconducting Oxide Composite Articles", assigned to the assignee of the present invention, and incorporated by reference. Other supercon-

ductors and their methods of fabrication are also described in co-pending application Ser. No. 08/554,814 filed on Nov. 7, 1995 by G. L. Snitchler, J. M. Seuntjens, W. L. Barnes and G. N. Riley, entitled "Cabled Conductors Containing Anisotropic Superconducting Compounds and Method for Making Them", assigned to the assignee of the present invention, and incorporated by reference. Ser. No. 08/719,987, filed Sep. 25, 1996, entitled "Decoupling of Superconducting Filaments in High Temperature Superconducting Composites," assigned to the assignee of the present invention, and incorporated by reference also describes methods of manufacturing superconducting wires well suited for conductor **22**.

In certain applications, the superconducting filaments and the matrix-forming material are encased in an insulating layer **30**. When the anisotropic superconducting material is formed into a tape, the critical current is often lower when the orientation of an applied magnetic field is perpendicular to the wider surface of the tape, as opposed to when the field is parallel to this wider surface. Conductor **22** of end regions **14** has a resistivity characteristic, in its normal state, less than that of conductor **18** of central region **11**.

Referring again to FIG. 2, electrical connections consisting of short lengths of conductive metal **34**, such as silver to join or splice the individual coils together in a series circuit. The individual coils can also be connected using conductive solder. In certain applications the short lengths of splicing material can be formed of superconducting material. A length of superconducting material (not shown) also connects one end of coil assembly **10** to a termination post located on end member **20** in order to supply current to coil assembly **10**. The current is assumed to flow in a counter-clockwise direction with the magnetic field vector **26** being generally normal to end member **18** (in the direction of longitudinal axis **31**) which forms the top of coil assembly **10**.

Although the embodiment described above in conjunction with FIG. 2 utilizes pancake type coils, other winding arrangements are within the scope of the claims. For example, referring to FIG. 7, a superconducting coil **40** includes a central region **42** wound with a tape **44** formed of an anisotropic superconductor material in layered arrangement. In a layered arrangement, tape **44** is wound along a longitudinal axis **46** of coil **40** from one end of coil **40** with successive windings wound next to the preceding winding until the opposite end of coil **40** is reached, thereby forming a first layer of the coil. Tape **44** is then wound back along axis **46** in the opposite direction and over the first layer of the coil. This winding approach is repeated until the desired number of turns is wound onto coil **40**. End regions **48** may be wound as a single or double pancake coil in the manner described above in conjunction with FIG. 2, or can be wound in a layered arrangement. End regions **48** are connected to central region **42** using metal or solder connections.

Referring to FIG. 8, in another embodiment, a superconducting coil **50** includes a central region **52** formed of high temperature anisotropic superconducting material wound in a layered arrangement. However, unlike coil **40** of FIG. 3, central region **50** is formed of individual lengths **54a**, **54b**, **54c** of high temperature anisotropic superconducting material. Each length **54a**, **54b**, **54c** is spliced (e.g., using solder or conductive metal joints) at end regions **56** to corresponding lengths **58a**, **58b**, **58c** of high temperature anisotropic superconducting material having the lower current density conductor.

Referring to FIG. 9, a superconducting transformer **60** includes a low voltage (high current) coil **62** and a high

voltage (low current) coil 64, each wound around iron cores (not shown) and on polymer tube mandrels 66. In this embodiment, low voltage coil 62 has four layers while high voltage coil has 20 layers. Each coil 62, 64 is contained within a cryogenic vessel (not shown) containing liquid nitrogen with the iron cores maintained at room temperature so that heat generated by the power dissipated in the cores is not transferred into the cryogenic vessel. In conjunction with the description above, both low voltage coil 62 and high voltage coil 64 include central region 66, 68 for providing current limiting, as well as end regions 70, 72, respectively, for maintaining a low AC loss performance in the presence of perpendicular magnetic fields at the end regions.

Depending on the particular application, each transformer design may have a different arrangement of superconductors used for central regions 66, 68 and end regions 70, 72. In one transformer embodiment rated at 30 MVA, end regions 70, 72 include 24 turns (12 at each end) of conductor while 51 turns of current limiting wire are provided for central regions 66, 68.

Referring to FIG. 10, a plot illustrating the RMS radial coil field (units of Tesla) as a function of the percent of the axial length of the coil, indicates that the radial magnetic field is almost nonexistent at the central region of the coils and increases dramatically at end regions. Thus, the current limiting wire in wire in monolithic form is generally provided only in central regions 66, 68 where the radial magnetic field is low.

In the table below, the relative performance of a transformer with and without low loss end regions is shown. The AC losses of a transformer having end regions 14 with conductor 22 can be fabricated with a lower aspect ratio wire to somewhat lower the losses. The low aspect monolith case shown in Table 1, has a change in the aspect ratio of the end-windings of a factor of about four. Thus, for certain applications, the transformer may include a conductor 22 having a low aspect ratio monolith.

| PARAMETER                                                           | High voltage | Low voltage | units     |
|---------------------------------------------------------------------|--------------|-------------|-----------|
| current rating                                                      | 157          | 787         | amp       |
| voltage rating                                                      | 110          | 20          | kilovolts |
| turns                                                               | 1500         | 300         |           |
| layers                                                              | 20           | 4           |           |
| total turns/layer                                                   | 75           | 75          |           |
| AC turns/layer                                                      | 24           | 24          |           |
| DC turns/layer                                                      | 51           | 51          |           |
| <hr/>                                                               |              |             |           |
| Maximum radial field                                                | 0.33         | 0.150       | tesla     |
| Maximum axial field                                                 | 0.240        | 0.240       | tesla     |
| AC heating without AC conductor                                     | 7.2          | 15.0        | mW/amp-m  |
| AC heating with AC conductor                                        | 1.7          | 1.7         | mW/amp-m  |
| AC heating with a low aspect ratio monolith replacing the AC turns. | 5.7          | 10.2        | mW/amp-m  |

What is claimed is:

1. A superconducting magnetic coil assembly having a center section and two end sections positioned along a longitudinal axis for generating a magnetic field that varies along the longitudinal axis of the coil assembly, the coil assembly comprising:

an anisotropic first superconductor wound about the longitudinal axis of the coil assembly in a region of the center section and forming a first coil section, the first superconductor having a first resistivity characteristic in a normal state of operation; and

a second superconductor wound about the longitudinal axis of the coil assembly in a region of at least one of the end sections and forming at least one second coil section, said second coil section connected in series to the first coil section, the second superconductor in a superconducting state of operation and in the presence of a magnetic field oriented perpendicular to the longitudinal axis, an AC loss characteristic of the second superconductor lower than an AC loss characteristic of the first superconductor, and

in a normal state of operation, a second resistivity characteristic of the second superconductor is less than the resistivity characteristic of the first anisotropic superconductor in a normal state of operation.

2. The superconducting magnetic coil of claim 1 wherein the second superconductor is connected to an end of the first anisotropic superconductor and is configured to provide a low AC loss characteristic in the presence of perpendicular magnetic fields.

3. The superconducting magnetic coil assembly of claim 1 wherein the second superconductor is formed of an anisotropic superconducting material.

4. The superconducting magnetic coil assembly of claim 3 wherein the first anisotropic superconductor is in the form of a superconductor tape.

5. The superconducting magnetic coil assembly of claim 4 wherein the first anisotropic superconductor tape is in a monolithic form.

6. The superconducting magnetic coil assembly of claim 5 wherein the monolithic-form first anisotropic superconductor tape is in the form of a monofilament superconductor.

7. The superconducting magnetic coil assembly of claim 5 wherein the monolithic-form first anisotropic superconductor tape includes a multifilament composite superconductor having individual superconducting filaments which extend the length of the multifilament composite superconductor.

8. The superconducting magnetic coil assembly of claim 7 wherein the first resistivity characteristic, in its normal state, is a range between about 10 to 50  $\mu\Omega\text{-cm}$ .

9. The superconducting magnetic coil assembly of claim 4 wherein the superconductor tape has an aspect ratio in a range between about 200:1 and 500:1.

10. The superconducting magnetic coil assembly of claim 4 wherein the superconductor tape includes a backing strip formed of a thermal stabilizer.

11. The superconducting magnetic coil assembly of claim 10 wherein the backing strip has a resistivity characteristic greater than about 10  $\mu\Omega\text{-cm}$ .

12. The superconducting magnetic coil assembly of claim 3 wherein the second anisotropic superconductor is formed as a superconductor tape.

13. The superconducting magnetic coil assembly of claim 12 wherein the superconductor tape of the second anisotropic superconductor includes a multifilament composite superconductor having individual superconducting filaments which extend the length of the multifilament composite superconductor and are surrounded by a matrix forming material.

14. The superconducting magnetic coil assembly of claim 13 wherein the individual superconducting filaments of the second anisotropic superconductor are twisted.

15. The superconducting magnetic coil assembly of claim 3 wherein the first superconductor is wound in a layered configuration.

16. The superconducting magnetic coil assembly of claim 3 wherein the first superconductor is formed of pancake coils each coil electrically connected to an adjacent coil.

17. The superconducting magnetic coil assembly of claim 16 wherein the first superconductor is formed of double pancake coils.

18. The superconducting magnetic coil assembly of claim 3 wherein the second superconductor is wound as a pancake coil.

19. The superconducting magnetic coil assembly of claim 15 wherein the second superconductor is wound as a pancake coil.

20. The superconducting magnetic coil assembly of claim 16 wherein the second anisotropic superconductor is wound as a pancake coil.

21. The superconducting magnetic coil assembly of claim 3 wherein a first segment of the first superconductor extends along the longitudinal axis in a first direction toward the second superconductor and connects to a first end of a first segment of the second superconductor at a first junction, a second end of the first segment connected to a second segment of the first superconductor, the second segment extending along the longitudinal axis in a second direction away from the second superconductor.

22. The superconducting magnetic coil assembly of claim 3 wherein the first and second superconductors are high temperature superconductors.

23. The superconducting magnetic coil assembly of claim 3 wherein the first superconductor constitutes greater than 50% of the total amount of superconductor of the coil.

24. The superconducting magnetic coil assembly of claim 3 wherein the second superconductor constitutes a portion of the total amount of superconductor of the coil in a range between 5% and 30%.

25. The superconducting magnetic coil assembly of claim 24 wherein the second superconductor constitutes about 10% of the total amount of superconductor of the coil.

26. A superconducting magnetic coil assembly having a center section and two end sections positioned along a longitudinal axis for generating a magnetic field that varies along the longitudinal axis of the coil assembly, the coil assembly comprising:

a first anisotropic superconductor wound about the longitudinal axis of the coil assembly in a region of the center section and forming a first coil section, the first anisotropic superconductor formed as a superconducting tape having a wide surface and configured to provide, in a superconducting state, a low AC loss characteristic in the presence of magnetic fields parallel to the wide surface of the superconducting tape; and

a second superconductor, different from the first anisotropic superconductor and wound about the longitudinal axis of the coil assembly in a region of at least one of the end sections and forming at least one second coil, the second superconductor connected to an end of the first anisotropic superconductor and configured to provide, in a superconducting state, a low AC loss characteristic in the presence of magnetic fields parallel to the wide surface of the superconducting tape of the first superconductor, wherein the AC loss characteristic of the second superconductor is lower than the AC loss characteristic of the first superconductor.

27. The superconducting magnetic coil assembly of claim 26 wherein the second superconductor is formed of an anisotropic superconducting material.

28. The superconducting magnetic coil assembly of claim 27 wherein the first anisotropic superconductor is in a monolithic form.

29. The superconducting magnetic coil assembly of claim 28 wherein the monolithic-form first anisotropic superconductor is in the form of a monofilament superconductor.

30. The superconducting magnetic coil assembly of claim 28 wherein the monolithic-form first anisotropic superconductor tape includes a multifilament composite superconductor having individual superconducting filaments which extend the length of the multifilament composite superconductor.

31. The superconducting magnetic coil assembly of claim 30 wherein the multifilament composite superconductor has a resistivity characteristic, in its normal state, in a range between about 10 to 50  $\mu\Omega\text{-cm}$ .

32. The superconducting magnetic coil assembly of claim 26 wherein the superconducting tape has an aspect ratio in a range between about 200:1 and 500:1.

33. The superconducting magnetic coil assembly of claim 26 wherein the superconducting tape includes a backing strip formed of a thermal stabilizer.

34. The superconducting magnetic coil assembly of claim 33 wherein the backing strip has a resistivity characteristic greater than about 10  $\mu\Omega\text{-cm}$ .

35. The superconducting magnetic coil assembly of claim 26 wherein the second anisotropic superconductor is formed as a superconducting tape.

36. The superconducting magnetic coil assembly of claim 35 wherein the second superconductor includes a multifilament composite superconductor having individual superconducting filaments which extend the length of the multifilament composite superconductor and are surrounded by a matrix forming material.

37. The superconducting magnetic coil assembly of claim 36 wherein the individual superconducting filaments of the second anisotropic superconductor are twisted.

38. The superconducting magnetic coil assembly of claim 26 wherein the first anisotropic superconductor is wound in a layered configuration.

39. The superconducting magnetic coil assembly of claim 26 wherein the first anisotropic superconductor is formed of pancake coils each coil electrically connected to an adjacent coil.

40. The superconducting magnetic coil assembly of claim 39 wherein the first superconductor is formed of double pancake coils.

41. The superconducting magnetic coil assembly of claim 26 wherein the second superconductor is wound as a pancake coil.

42. The superconducting magnetic coil assembly of claim 38 wherein the second superconductor is wound as a pancake coil.

43. The superconducting magnetic coil assembly of claim 38 wherein the second superconductor is wound as a pancake coil.

44. The superconducting magnetic coil assembly of claim 26 wherein a first segment of the first superconductor extends along the longitudinal axis in a first direction toward the second superconductor and connects to a first end of a first segment of the second superconductor at a first junction, a second end of the first segment connected to a second segment of the first superconductor, the second segment extending along the longitudinal axis in a second direction away from the second superconductor.

**11**

**45.** The superconducting magnetic coil assembly of claim **26** wherein the first and second superconductors are high temperature superconductors.

**46.** The superconducting magnetic coil assembly of claim **26** wherein the first superconductor constitutes greater than <sup>5</sup> 50% of the total amount of superconductor of the coil.

**47.** The superconducting magnetic coil assembly of claim **26** wherein the second superconductor constitutes a portion of the total amount of superconductor of the coil in a range between 5% and 30%. <sup>10</sup>

**48.** The superconducting magnetic coil assembly of claim **47** herein the second superconductor constitutes about 10% of the total amount of superconductor of the coil.

**49.** A superconducting magnetic coil assembly generating a magnetic field that varies along a longitudinal axis, the coil <sup>15</sup> assembly comprising:

**12**

a center coil section wound about the longitudinal axis in a center region of the coil assembly and comprising a first anisotropic superconductor; and

at least one end coil section wound about the longitudinal axis in an end region of the coil assembly, said end coil section positioned proximate to the center coil section along the longitudinal axis and comprising a second superconductor different from said first anisotropic superconductor;

wherein said second superconductor has lower AC losses in the presence of a magnetic field oriented perpendicular to the longitudinal axis than said first anisotropic superconductor.

\* \* \* \* \*